

## UNITED STATES PATENT OFFICE

2,029,156

## OXIDE FLOTATION

Ludwig J. Christmann, Jersey City, and Stuart A. Falconer, Elizabeth, N. J., assignors to American Cyanamid Company, New York, N. Y., a corporation of Maine

No Drawing. Application November 1, 1928,  
Serial No. 316,610

4 Claims. (Cl. 209—166)

This discovery relates to a process of recovering values from oxide ores as distinguished from those of the sulfide type.

Throughout this specification the terms "oxidized ore", "oxide ore" or "non-sulfide ore" are intended to designate an ore in which the metal values are present substantially as non-sulfide compounds. In such ores the metal values may occur as carbonate, sulfate, oxide, or as some other oxygenated compound of the metal. Such ores have usually been formed in nature by oxidation of the original sulfides, and consequently, they may contain small amounts of unaltered sulfides. As far as the present discovery is concerned, however, such sulfides are present incidentally.

The recovery of sulfide minerals by the flotation process is now highly developed and reagents adapted thereto are well known in the art. Heretofore, however, the flotation concentration of oxide ores has been very unsatisfactory. Practically all of the proposed methods have involved a preliminary sulfidization of the oxide component in an attempt to produce upon the surface of the mineral a coating of sulfide which would render it susceptible to ordinary sulfide flotation reagents. This sulfidization operation has proven very troublesome in practice, partly because some of the oxide minerals sulfidize with difficulty, if at all, and partly because the sulfidizing reagent frequently introduces complications and difficulties in the operation of the flotation cell.

The essence of the invention is that such oxide minerals are recovered without preliminary sulfidization by employing a reagent or combination of reagents adapted specifically to the flotation of such oxide minerals.

Although certain of the reagents specified in this application are well known in the recovery of sulfides, it does not follow that sulfide reagents are applicable to oxide flotation, and, as a matter of fact, there is no theory of reasoning by which one could conclude that a sulfide flotation reagent would operate efficiently with oxides. The entire history of the flotation art has shown that the reverse is true. According to prior practice, values present in non-sulfide form were either recovered by sulfidization or were lost with the tailings. In the present invention, however, by suitable selection of reagents, the non-sulfide minerals may be recovered by froth flotation by the use of a reagent combination adapted to the recovery of such specific minerals.

The reagents employed in flotation serve a number of specific purposes and may in general be divided into three classes: first, collectors or pro-

moters whose function is to collect into aggregates the mineral to be floated, and probably to attach such aggregates to the bubble; second, frothing agents whose purpose is to supply the bubble which is essential for the raising of the heavy mineral particles from the ore pulp; and third, reagents known as conditioning reagents whose exact function is obscure but which probably serve a variety of purposes such as freeing the solution from soluble heavy metal salts which, if not so removed, would themselves consume the more expensive collectors, and possibly also to establish a proper hydrogen-ion concentration.

The use of such collectors as potassium ethyl xanthate, thiocarbanilid and the dithiophosphates is old in the flotation of sulfide minerals. As has been stated above and as is shown in the results which follow, such collecting reagents are not themselves well adapted to the flotation of oxide minerals except when used in conjunction with certain other reagents as disclosed herein.

As frothing agents, such materials as pine oil and cresylic acid are usually employed. Frequently the collector itself has frothing properties, in which case it may be unnecessary to add any specific frothing agent. This is particularly true where oxidized ores are under consideration, since these almost always froth more readily than sulfides. In many of the examples given in this specification, no auxiliary frothing agent has been used, the frothing properties being derived from the collector. In some cases, however, the use of small amounts of frothing agent may be found advantageous.

The use of acids and alkalies as modifying agents is old in the flotation art. As has been shown above, their function is to regulate the hydrogen-ion concentration and frequently to precipitate soluble salts from solution. As preferred modifying agents there may be used acids whose heavy metal salts are insoluble, and oxalic, sulfuric and particularly phosphoric acid have been found to be effective. The only explanation of the action of these modifying agents is that their function is to convert the metal or metals to be recovered into a form which makes them more readily collected by the reagent combinations which are employed.

One of the important features of this discovery is that oxides are particularly amenable to flotation in the presence of a mercaptothiazole or derivatives thereof, either with or without frothing agents. It has also been found that good results are obtained in oxide flotation by combining a mercaptothiazole or its derivative with other

well or lesser known flotation reagents, the result being considerably more efficient than either reagent used alone.

Among the reagents which have been found efficient are: the mercaptothiazoles, mercaptobenzothiazoles and particularly the sodium salt thereof, 4 methyl and 6 chlor mercaptobenzothiazole, dithiophosphoric acids, the disubstituted dithiophosphoric acids and particularly the sodium salt of diisopropylidithiophosphoric acid, as well as the ammonium and aniline salts thereof, mixtures of soda ash and a disubstituted dithiophosphoric acid, the alkyl xanthates, particularly amyl xanthate, and the potassium salts thereof and mixtures of cresylic acid and the disubstituted dithiophosphoric acids such as the diaryldithiophosphoric acids.

Tests have shown the efficacy of these reagents and combinations thereof in the recovery of copper, lead, silver and gold.

In Table No. 1 the ore was from one of the properties of the International Smelting Company in Utah and known as the North Lily mine, which analyzed as follows:

|    |                  |  | Per cent |
|----|------------------|--|----------|
| 25 | Total lead       |  | 29.60    |
|    | Non-sulfide lead |  | 25.93    |
|    | Total zinc       |  | 0.53     |
|    | Non-sulfide zinc |  | 0.45     |
| 30 | Iron             |  | 6.96     |
|    | Sulfur           |  | 4.90     |
|    | Insoluble        |  | 42.35    |
|    | CaO              |  | 1.33     |
|    | MgO              |  | 0.28     |
| 35 | Cu               |  | 0.065    |
|    | Au, oz./ton      |  | 0.155    |
|    | Ag, oz./ton      |  | 11.93    |

The flotation results on copper, listed in Table No. 2 were had from tests made upon ore from

40

The Bagdad Copper Company which analyzed as follows:

|                    | Per cent |
|--------------------|----------|
| Total copper       | 3.27     |
| Non-sulfide copper | 3.07     |
| Iron               | 2.52     |
| Insoluble          | 82.4     |

Unless otherwise noted the procedure was substantially as follows:

Approximately 1200 grams of ore were ground with 1200 grams of water with or without a reagent in a rod mill for 10 minutes. The pulp was then transferred to a laboratory, mechanically agitated, flotation cell and diluted to 22% solids. This pulp was then subjected to a flotation operation for the time indicated.

In the tables, the following abbreviations are used to indicate the reagents:

MMBT—4 methyl mercaptobenzothiazole  
CMBT—6 chlor mercaptobenzothiazole

NaMBT—Sodium salt of mercaptobenzothiazole  
NaDIPDTP—Sodium salt of diisopropylidithiophosphoric acid, an 85% product was used.

NH<sub>4</sub>DIPDTP—Ammonium salt of diisopropylidithiophosphoric acid

NaAF30—Mixture of soda ash (50% by weight) and the sodium salt of diethylidithiophosphoric acid

Aero-X—Aniline salt of diisopropylidithiophosphoric acid

KAX—Potassium amyl xanthate  
KBX—Potassium butyl xanthate

KEX—Potassium ethyl xanthate  
AF15—Mixture of cresylic acid (40% by weight) and dicesyldithiophosphoric acid

S. B. F. O.—Scotch blast furnace oil

In all cases, either the collector imparted frothing properties to the pulp, or else sufficient frother was added.

Table No. 1

| 45 | Test no. | Weight       |              | Concentrates     |        |        | To rod mill    |                                | Reagent in lbs. per ton                 |                                         |                         |                         | Time of float (min.) |
|----|----------|--------------|--------------|------------------|--------|--------|----------------|--------------------------------|-----------------------------------------|-----------------------------------------|-------------------------|-------------------------|----------------------|
|    |          | Conc. (gms.) | Tails (gms.) | Percent Pb Grade | Ag oz. | Au oz. | Pounds per ton | Re-agent                       | Start                                   | 5 min.                                  | 10 min.                 | 15 min.                 |                      |
|    |          |              |              | Recov.           | Recov. | Recov. |                |                                | Recov.                                  | Recov.                                  | Recov.                  | Recov.                  |                      |
| 50 | 3        | 457          | 711          | 62.9             | 29.53  | 0.42   | 5              | H <sub>3</sub> PO <sub>4</sub> | 1.0 NaMBT<br>1.0 Aero-X                 | 0.5 NaMBT<br>0.5 Aero-X                 | -----                   | -----                   | 15 50                |
|    |          |              |              | 85.0             | 87.1   | 77.4   |                |                                | -----                                   | -----                                   | -----                   | -----                   |                      |
| 55 | 4        | 520          | 646          | 57.8             | 26.44  | 0.245  | 1              | H <sub>3</sub> PO <sub>4</sub> | 1.0 NaMBT<br>1.0 Aero-X                 | 0.5 NaMBT<br>0.5 Aero-X                 | 0.5 NaMBT<br>0.5 Aero-X | 0.5 NaMBT<br>0.5 Aero-X | 20                   |
|    |          |              |              | 91.5             | 91.5   | 73.0   |                |                                | -----                                   | -----                                   | -----                   | -----                   |                      |
| 60 | 5        | 430          | 735          | 61.2             | 28.85  | 0.25   | 3              | H <sub>3</sub> PO <sub>4</sub> | do                                      | do                                      | do                      | do                      | 20 55                |
|    |          |              |              | 82.0             | 84.4   | 61.9   |                |                                | -----                                   | -----                                   | -----                   | -----                   |                      |
| 65 | 6        | 527          | 647          | 57.4             | 25.65  | 0.255  | 5              | H <sub>3</sub> PO <sub>4</sub> | do                                      | do                                      | do                      | do                      | 20                   |
|    |          |              |              | 91.0             | 90.5   | 73.4   |                |                                | -----                                   | -----                                   | -----                   | -----                   |                      |
| 70 | 7        | 470          | 705          | 62.9             | 29.54  | 0.26   | 5              | H <sub>3</sub> PO <sub>4</sub> | 1.0 NaMBT<br>0.5 NH <sub>4</sub> DIPDTP | 1.0 NaMBT<br>0.5 NH <sub>4</sub> DIPDTP | -----                   | -----                   | 15 60                |
|    |          |              |              | 88.0             | 87.8   | 65.9   |                |                                | -----                                   | -----                                   | -----                   | -----                   |                      |
| 75 | 8        | 424          | 727          | 66.6             |        |        | 5              | H <sub>3</sub> PO <sub>4</sub> | 1.0 NaMBT<br>0.5 NaDIP-DTP              | 1.0 NaMBT<br>0.5 NaDIP-DTP              | -----                   | -----                   | 15                   |
|    |          |              |              | 85.2             |        |        |                |                                | -----                                   | -----                                   | -----                   | -----                   |                      |
| 80 | 9        | 270          | 898          | 57.6             |        |        | 6              | H <sub>2</sub> SO <sub>4</sub> | 1.0 NaMBT<br>1.0 Aero-X                 | 0.5 NaMBT<br>0.5 Aero-X                 | 0.5 NaMBT<br>0.5 Aero-X | 0.5 NaMBT<br>0.5 Aero-X | 20 65                |
|    |          |              |              | 46.5             |        |        |                |                                | -----                                   | -----                                   | -----                   | -----                   |                      |
| 85 | 10       | 426          | 753          | 58.3             |        |        | 3              | H <sub>2</sub> SO <sub>4</sub> | do                                      | do                                      | do                      | do                      | 20                   |
|    |          |              |              | 70.7             |        |        |                |                                | -----                                   | -----                                   | -----                   | -----                   |                      |
| 90 | 11       | 532          | 633          | 56.7             | 26.98  | 0.26   | 1              | H <sub>2</sub> SO <sub>4</sub> | do                                      | do                                      | do                      | do                      | 20 70                |
|    |          |              |              | 88.0             | 88.4   | 74.0   |                |                                | -----                                   | -----                                   | -----                   | -----                   |                      |
| 95 | 12       | 603          | 566          | 49.8             | 23.48  | 0.22   | 3              | H <sub>2</sub> SO <sub>4</sub> | do                                      | do                                      | do                      | do                      | 20                   |
|    |          |              |              | 86.0             | 88.0   | 74.2   |                |                                | -----                                   | -----                                   | -----                   | -----                   |                      |

Table No. 1—Continued

| 5  | Test no. | Weight       |              | Concentrates     |        |        | To rod mill    |                                             | Reagent in lbs. per ton              |                                      |                                      |                            | Time of float (min.) |
|----|----------|--------------|--------------|------------------|--------|--------|----------------|---------------------------------------------|--------------------------------------|--------------------------------------|--------------------------------------|----------------------------|----------------------|
|    |          | Conc. (gms.) | Tails (gms.) | Percent Pb Grade | Ag oz. | Au oz. | Pounds per ton | Reagent                                     | Start                                | 5 min.                               | 10 min.                              | 15 min.                    |                      |
|    |          |              |              | Recov.           | Recov. | Recov. |                |                                             | do                                   | do                                   | do                                   | do                         |                      |
| 10 | 13       | 537          | 631          | 57.3             | 24.46  | 0.24   | 1              | Oxalic                                      | do                                   | do                                   | do                                   | do                         | 5                    |
|    |          |              |              | 86.0             | 83.9   | 69.4   |                |                                             | do                                   | do                                   | do                                   | do                         |                      |
| 14 | 14       | 329          | 829          | 59.7             |        |        | 3              | do                                          | do                                   | do                                   | do                                   | do                         | 20                   |
|    |          |              |              | 55.6             |        |        |                |                                             | do                                   | do                                   | do                                   | do                         |                      |
| 15 | 15       | 258          | 910          | 59.3             |        |        | 5              | do                                          | do                                   | do                                   | do                                   | do                         | 15                   |
|    |          |              |              | 44.6             |        |        |                |                                             | do                                   | do                                   | do                                   | do                         |                      |
| 16 | 16       | 180          | 970          | 37.5             |        |        | 5              | H <sub>3</sub> PO <sub>4</sub>              | 1.0 Aero-X<br>0.08 AF15              | 1.0 Aero-X<br>0.08 AF15              | 0.08 AF15                            |                            | 20                   |
|    |          |              |              | 20.4             |        |        |                |                                             | do                                   | do                                   | do                                   | do                         |                      |
| 20 | 17       | 184          | 985          | 45.3             |        |        | 5              | H <sub>3</sub> PO <sub>4</sub>              | 1.0 Aero-X<br>0.08 AF15              | 1.0 Aero-X<br>0.08 AF15              | 1.0 Aero-X<br>0.08 AF15              | 1.0 Aero-X<br>0.08 AF15    | 20                   |
|    |          |              |              | 24.4             |        |        |                |                                             | do                                   | do                                   | do                                   | do                         |                      |
| 25 | 18       | 194          | 989          | 63.2             |        |        | 5              | H <sub>3</sub> PO <sub>4</sub>              | 1.0 NaMBT<br>0.08 AF15               | 1.0 NaMBT<br>0.08 AF15               | 0.08 AF15                            |                            | 20                   |
|    |          |              |              | 36.3             |        |        |                |                                             | do                                   | do                                   | do                                   | do                         |                      |
| 25 | 19       | 325          | 843          | 61.2             |        |        | 5              | H <sub>3</sub> PO <sub>4</sub>              | 1.0 NaMBT<br>0.08 AF15               | 1.0 NaMBT<br>0.08 AF15               | 1.0 NaMBT<br>0.08 AF15               | 1.0 NaMBT<br>0.08 AF15     | 20                   |
|    |          |              |              | 57.0             |        |        |                |                                             | do                                   | do                                   | do                                   | do                         |                      |
| 30 | 20       | 197          | 975          | 42.6             |        |        | 5              | H <sub>3</sub> PO <sub>4</sub>              | 1.0 NaDIP-DTP<br>0.08 AF15           | 1.0 NaDIP-DTP<br>0.08 AF15           |                                      |                            | 20                   |
|    |          |              |              | 25.2             |        |        |                |                                             | do                                   | do                                   | do                                   | do                         |                      |
| 30 | 21       | 387          | 811          | 60.7             |        |        | 5              | H <sub>3</sub> PO <sub>4</sub>              | 1.0 NaDIP-DTP<br>0.08 AF15           | 1.0 NaDIP-DTP<br>0.08 AF15           | 1.0 NaDIP-DTP<br>0.08 AF15           | 1.0 NaDIP-DTP<br>0.08 AF15 | 20                   |
|    |          |              |              | 65.8             |        |        |                |                                             | do                                   | do                                   | do                                   | do                         |                      |
| 35 | 22       | 265          | 896          | 67.0             |        |        | 5              | H <sub>3</sub> PO <sub>4</sub>              | 1.0 NaMBT<br>1.0 NaAF30              | 0.5 NaMBT<br>0.5 NaAF30              | 0.5 NaMBT<br>0.5 NaAF30              |                            | 20                   |
|    |          |              |              | 53.3             |        |        |                |                                             | do                                   | do                                   | do                                   | do                         |                      |
| 35 | 23       | 572          | 637          | 54.85            | 25.16  | 0.24   | 5              | H <sub>3</sub> PO <sub>4</sub>              | 1.0 NaMBT<br>1.0 NaDIP-DTP           | 0.5 NaMBT<br>0.5 NaDIP-DTP           | 0.5 NaMBT<br>0.5 NaDIP-DTP           |                            | 35                   |
|    |          |              |              | 88.5             | 88.5   | 75.5   |                |                                             | do                                   | do                                   | do                                   | do                         |                      |
| 40 | 24       | 479          | 702          | 65.8             | 30.14  | 0.27   | 5              | H <sub>3</sub> PO <sub>4</sub>              | 1.0 NaMBT<br>1.0 KAX                 | 0.5 NaMBT<br>0.5 KAX                 | 0.5 NaMBT<br>0.5 KAX                 |                            | 20                   |
|    |          |              |              | 90.0             | 88.4   | 69.8   |                |                                             | do                                   | do                                   | do                                   | do                         |                      |
| 45 | 25       | 259          | 900          | 63.6             |        |        | 5              | H <sub>3</sub> PO <sub>4</sub>              | 2.0 KBX<br>2.0 NaMBT                 | 0.04 AF15                            | 0.04 AF15                            |                            | 20                   |
|    |          |              |              | 48.4             |        |        |                |                                             | do                                   | do                                   | do                                   | do                         |                      |
| 45 | 26       | 353          | 827          | 64.8             |        |        | 5              | H <sub>3</sub> PO <sub>4</sub>              | 2.0 NaMBT<br>2.0 KEX<br>0.04 AF15    | 0.04 AF15                            | 0.04 AF15                            |                            | 45                   |
|    |          |              |              | 67.8             |        |        |                |                                             | do                                   | do                                   | do                                   | do                         |                      |
| 50 | 27       | 112          | 1055         | 52.4             |        |        | 5              | H <sub>3</sub> PO <sub>4</sub>              | 1.0 NaMBT<br>0.04 AF15               | 1.0 NaMBT                            | 1.0 NaMBT<br>0.04 AF15               |                            | 20                   |
|    |          |              |              | 17.7             |        |        |                |                                             | do                                   | do                                   | do                                   | do                         |                      |
| 50 | 28       | 276          | 825          | 34.1             |        |        | 5              | H <sub>3</sub> PO <sub>4</sub>              | 1.0 Aero-X<br>0.04 AF15              | 1.0 Aero-X                           | 1.0 Aero-X<br>0.02 AF15              | 1.0 Aero-X<br>0.02 AF15    | 20                   |
|    |          |              |              | 28.0             |        |        |                |                                             | do                                   | do                                   | do                                   | do                         |                      |
| 50 | 30       | 199          | 932          | 37.6             |        |        | 5              | H <sub>3</sub> PO <sub>4</sub>              | 1.0 KAX                              | 1.0 KAX                              | 1.0 KAX                              | 1.0 KAX                    | 20                   |
|    |          |              |              | 21.9             |        |        |                |                                             | do                                   | do                                   | do                                   | do                         |                      |
| 55 | 31       | 86           | 1082         | 43.6             |        |        | 5              | H <sub>3</sub> PO <sub>4</sub>              | 1.0 KAX<br>0.04 AF15                 | 1.0 KAX                              | 1.0 KAX                              | 1.0 KAX                    | 20                   |
|    |          |              |              | 11.2             |        |        |                |                                             | do                                   | do                                   | do                                   | do                         |                      |
| 55 | 32       | 256          | 912          | 41.9             |        |        | 5              | H <sub>3</sub> PO <sub>4</sub>              | 1.0 NaDIP-DTP                        | 1.0 NaDIP-DTP                        | 1.0 NaDIP-DTP                        | 1.0 NaDIP-DTP              | 20                   |
|    |          |              |              | 31.6             |        |        |                |                                             | do                                   | do                                   | do                                   | do                         |                      |
| 60 | 33       | 435          | 719          | 38.0             |        |        | 5              | H <sub>3</sub> PO <sub>4</sub>              | 1.0 KAX<br>1.0 NaDIP-DTP             | 0.5 KAX<br>0.5 NaDIP-DTP             | 0.5 KAX<br>0.5 NaDIP-DTP             |                            | 60                   |
|    |          |              |              | 49.2             |        |        |                |                                             | do                                   | do                                   | do                                   | do                         |                      |
| 65 | 34       | 212          | 966          | 38.9             |        |        | 5              | H <sub>3</sub> PO <sub>4</sub>              | 1.0 KBX<br>1.0 NaDIP-DTP             | 0.5 KBX<br>0.5 NaDIP-DTP             | 0.5 KBX<br>0.5 NaDIP-DTP             |                            | 20                   |
|    |          |              |              | 24.0             |        |        |                |                                             | do                                   | do                                   | do                                   | do                         |                      |
| 65 | 35       | 387          | 788          | 63.65            |        |        | 2              | Thiocarbamid H <sub>3</sub> PO <sub>4</sub> | 1.0 NaMBT                            | 0.5 NaMBT<br>0.04 AF15               | 0.5 NaMBT<br>0.04 AF15               |                            | 65                   |
|    |          |              |              | 70.7             |        |        |                |                                             | do                                   | do                                   | do                                   | do                         |                      |
| 70 | 36       | 342          | 826          | 67.83            |        |        | 5              | H <sub>3</sub> PO <sub>4</sub>              | 1.0 NaMBT<br>1.0 TEXACA<br>0.04 AF15 | 0.5 NaMBT<br>0.5 TEXACA<br>0.04 AF15 | 0.5 NaMBT<br>0.5 TEXACA<br>0.04 AF15 |                            | 20                   |
|    |          |              |              | 67.0             |        |        |                |                                             | do                                   | do                                   | do                                   | do                         |                      |
| 70 | 41       | 510          | 650          | 62.5             | 26.42  | 0.20   | 5.0            | H <sub>3</sub> PO <sub>4</sub>              | 1.0 MMBT<br>1.0 KAX                  | 0.5 MMBT<br>0.5 KAX                  | 0.5 MMBT<br>0.5 KAX                  |                            | 20                   |
|    |          |              |              | 94.0             | 91.3   | 69.2   |                |                                             | do                                   | do                                   | do                                   | do                         |                      |
| 75 | 42       | 510          | 670          | 63.5             | 25.80  | 0.20   | 5.0            | H <sub>3</sub> PO <sub>4</sub>              | 1.0 CMBT<br>1.0 KAX                  | 0.5 CMBT<br>0.5 KAX                  | 0.5 CMBT<br>0.5 KAX                  |                            | 20                   |
|    |          |              |              | 92.2             | 89.3   | 68.5   |                |                                             | do                                   | do                                   | do                                   | do                         |                      |

Table No. 1—Continued

| 5  | Test no. | Weight       |              | Concentrates     |        |        | To rod mill    |           | Reagent in lbs. per ton |          |          |          | Time of float (min.) |
|----|----------|--------------|--------------|------------------|--------|--------|----------------|-----------|-------------------------|----------|----------|----------|----------------------|
|    |          | Conc. (gms.) | Tails (gms.) | Percent Pb Grade | Ag oz. | Au oz. | Pounds per ton | Reagent   | Start                   | 5 min.   | 10 min.  | 15 min.  |                      |
|    |          |              |              | Recov.           | Recov. | Recov. |                |           |                         |          |          |          |                      |
| 10 | 43       | 460          | 712          | 58.35            | 26.02  | 0.19   | 5.0            | $H_3PO_4$ | 1.0 CMBT<br>0.20 Tarol  | 1.0 CMBT | 1.0 CMBT | 1.0 CMBT | 20 10                |
|    |          |              |              | 77.7             | 79.1   | 60.5   |                |           |                         |          |          |          |                      |
| 44 | 480      | 702          |              | 64.10            | 26.60  | 0.20   | 5.0            | $H_3PO_4$ | 1.0 MMBT<br>0.20 Tarol  | 1.0 MMBT | 1.0 MMBT | 1.0 MMBT | 20                   |
|    |          |              |              | 89.1             | 86.4   | 64.6   |                |           |                         |          |          |          |                      |

15

Table No. 2

| 20  | Test no. | Weight      |             | Conc.            | Tails            | To rod mill  |         | Reagent in lbs. per ton |        | Time of float (min.) |  |
|-----|----------|-------------|-------------|------------------|------------------|--------------|---------|-------------------------|--------|----------------------|--|
|     |          | Conc. (gms) | Tails (gms) | Percent Cu Grade | Percent Cu Grade | Lbs. per ton | Reagent | Start                   | 5 min. |                      |  |
|     |          |             |             | Recov.           | Recov.           |              |         |                         |        |                      |  |
| 127 | 127      | 95          | 1073        | 24.19            | 2.12             | 1            | SBFO    | 1.0 NaMBT               |        | 15                   |  |
|     |          |             |             | 50.2             | 49.8             |              |         |                         |        |                      |  |
| 25  | 128      | 168         | 1005        | 17.81            | 1.35             | 2            | SBFO    | 1.0 NaMBT<br>.2 TAROL   |        | 25                   |  |
|     |          |             |             | 65.8             | 31.2             |              |         |                         |        |                      |  |
| 30  | 129      | 230         | 951         | 13.51            | 1.41             | 4            | SBFO    | 2.0 NaMBT               |        | 15                   |  |
|     |          |             |             | 69.8             | 30.2             |              |         |                         |        |                      |  |

Tests 6, 12, 17, 19, 27 and 28 show the effect on oxide recovery of the mercaptothiazoles in natural and phosphoric acid circuits, together with the effect of Aero-X in natural and phosphoric acid circuits, and both reagents in combination. A comparison of these tests shows the remarkable effect of NaMBT on oxide ore in the presence of Aero-X. It also appears that phosphoric acid increases the oxide grade appreciably.

Tests 9, 10, 11 and 12 were made to determine the effect of sulfuric acid on oxide grade and recovery in a circuit including NaMBT and Aero-X. These tests show that a small amount of sulfuric acid increases the grade of concentrate without increasing recovery appreciably, and that large amounts of sulfuric acid do not further increase the grade but on the other hand, do materially effect recovery.

Tests 12, 13, 14 and 15 demonstrate the effect of oxalic acid as a typical organic acid on oxide grade and recovery, using the same reagents as above. These tests show that a small amount of oxalic acid increases the grade without increasing recovery and that larger amounts of this acid cause a falling off of recovery without, however, affecting the grade.

Tests 4, 5, 6 and 12 were made in much the same manner using phosphoric acid as the reagent in the rod mill. These tests show that phosphoric acid materially increases the grade and gives some increase in recovery. The phosphoric acid added even in equivalents of as much as 5 pounds per ton do not cause a decrease in recovery, so that phosphoric acid is to be preferred as compared with sulfuric or oxalic acids.

A comparison of tests 8, 19, 21, 27 and 32 shows the effect of NaDIPDTP, alone, NaMBT both alone and together using AF15 as a frother. These tests clearly show that the combination of NaMBT and NaDIPDTP is better than either alone and remarkable results are had from this combination.

Tests 16, 17 and 28 show the effect of one of the disubstituted dithiophosphoric acids, and

particularly the aniline salt of the diisopropyl form with sufficient frother, in both natural and acid circuits, on lead recovery. They show that with Aero-X a natural circuit gives somewhat poorer grade but slightly better recovery, and that even large amounts of Aero-X do not appreciably increase recovery.

Tests 20, 21 and 32 demonstrate the effect of the disubstituted dithiophosphoric acids, using AF15 in both natural and acid circuits. These tests seem to indicate that with sodium diisopropylthiophosphoric acid, free phosphoric acid increases both grade and recovery. Large amounts of the flotation reagent in acid circuit give an appreciable recovery.

Tests 6, 7, 8 and 22 were made to study the effect of the mercaptothiazoles in combination with various members of the disubstituted dithiophosphoric derivatives in phosphoric acid circuits. These tests clearly show that good flotation combinations may be had with these reagents.

Tests 19, 24, 27, 30 and 31 demonstrate the effect on oxide recovery of KAX and NaMBT alone using AF15, and in combination, in natural and phosphoric acid circuits. From these tests it would conclusively appear that the combination of NaMBT and KAX is better than either alone.

Tests 41 and 42 show the beneficial effects of other mercaptobenzothiazoles in combination with KAX.

A run was made following the procedure of test 24, using only one pound  $H_3PO_4$  per ton in the rod mill, the grind being carried out to the following point:

|            | Per cent |
|------------|----------|
| + 65 mesh  | 0.25     |
| + 100 mesh | 1.40     |
| + 150 mesh | 3.25     |
| + 200 mesh | 8.10     |
| - 200 mesh | 87.00    |

This test recovered 96% Pb of a 58.04% grade, 93.3% Ag of a grade of 25.83 oz. per ton, and

76.0% Au of a grade of 0.21 oz. per ton. These results show increased recovery may be had by grinding as above, although there is a slight decrease in grade.

5 A lesser grind in which 74.30% passed a 200 mesh screen recovered 95.9% Pb of a 60.18% grade.

Following the procedure of test 6, but grinding in the rod mill until 74.75% passed a 200 mesh screen, 95.2% Pb was recovered in a froth of a 51.31% grade. This confirms the deduction as to the effect of grinding, as made in connection with the test compared with test 24.

A comparison of tests 24, 25 and 26 shows the 15 effect of the mercaptobenzothiazoles in combination with various members of the alkyl xanthate series in phosphoric acid on oxide recovery. These tests appear to indicate that the potency of the various xanthates with sodium mercaptobenzothiazole are in the following order: KAX—KEX—KBX.

The effect of various reagents plus sodium mercaptobenzothiazole in phosphoric acid circuits is shown in tests 34, 35 and 36.

25 Tests 43 and 44 show excellent recovery with various thiiazoles using tarol as a frother.

A comparison of tests 21, 31 and 33 seems to indicate that sodium diisopropylthiophosphoric acid with AF15 as a frother is a better reagent than the combination KAX, and NADIPDTP.

The effect of the alkyl xanthates above in natural circuit and using AF15 in phosphoric acid circuits, on oxide recovery, is shown in tests 30 and 31. There it is found that in an acid circuit 30 with AF15, grade is increased slightly and recovery decreased. In either natural or acid circuit recovery may be had by KAX alone.

A comparison of tests 3, 4, 5, 6, 7, 11, 12, 13, 23 and 24 shows the remarkable recovery had on 40 silver and gold as well as the lead from oxide ore. These tests would seem to indicate that the recovery of lead and silver runs substantially par-

allel, and exceptionally good results as to total recovery may also be had by the use of these reagents.

From a comparison of tests 27, 28 and 29 it will be seen that as much as 69% of the copper can be 5 recovered in a grade averaging 18%, with sodium mercaptobenzothiazole, Scotch blast furnace oil and tarol.

It is to be clearly understood that the results here tabulated are merely indicative as to the 10 types of reagents and reagent combinations which will float oxide ores. Obviously the amounts of reagents specified are not considered absolutely necessary, and it is distinctly understood that this discovery is not limited to the proportions indicated. The discovery lies principally in the fact that certain reagents may be used with exceptional advantage in flotation processes for the recovery of the heavy metals from oxide ores.

We claim:

1. A method of concentrating oxidized ores which includes the step of subjecting an oxidized ore to a froth flotation operation in the presence of a mercaptobenzothiazole, a diisopropylthiophosphoric acid salt and phosphoric acid. 20

2. A method of concentrating oxidized ores which includes the step of subjecting an oxidized ore to a froth flotation operation in the presence of sodium mercaptobenzothiazole, sodium diisopropylthiophosphate and phosphoric acid. 25

3. A method of concentrating oxidized ores which includes the step of subjecting an oxidized ore to a froth flotation operation in the presence of sodium mercaptobenzothiazole, phosphoric acid and a frother. 30

4. A method of concentrating oxidized ores which includes the step of subjecting an oxidized ore to a froth flotation operation in the presence of a mercaptobenzothiazole, a frother and phosphoric acid. 40

LUDWIG J. CHRISTMANN.  
STUART A. FALCONER.